

Sept. 29, 1970

E. N. URFER ET AL

3,531,694

VOLTAGE-SENSITIVE SWITCH

Filed July 18, 1968



1

3,531,694

## VOLTAGE-SENSITIVE SWITCH

Ernest N. Urfer, North Adams, John J. Randall, Jr., Williamstown, and Henry F. Puppolo, North Adams, Mass., assignors to Sprague Electric Company, North Adams, Mass., a corporation of Massachusetts

Filed July 18, 1968, Ser. No. 745,879

Int. Cl. H01g 3/075

U.S. Cl. 317—230

15 Claims

### ABSTRACT OF THE DISCLOSURE

A counterelectrode overlies the anodic oxide layer formed on the surface of an aluminum electrode. The aluminum electrode contains at least one isolated, visible iron-containing impurity site. The voltage-sensitive switch is formed by chemically or electro-chemically cleaning and polishing an aluminum electrode, treating the cleaned and polished electrode with a hydroxyl-containing polar compound, preferably water, for a period sufficient to make the iron-containing impurity site latently visible, anodizing the treated surface in chromic acid to form an anodic oxide layer which reveals said iron-containing impurity site, and applying a counterelectrode. The method can also be employed to determine the presence or absence of iron-containing impurity sites in aluminum.

### BACKGROUND OF THE INVENTION

The present invention is concerned with a voltage-sensitive switch and a method for forming the same. The invention is also concerned with a method for determining the presence or absence of iron-containing impurity sites in aluminum.

The voltage-sensitive switch is a thin film solid state device which is designed to short circuit when a pulse voltage of predetermined amplitude is applied across its terminals. Switches of this type are described in co-pending U.S. patent application S.N. 326,152, filed Nov. 26, 1963 in the names of Henry F. Puppolo et al., now Pat. 3,412,220. The switch defined in this co-pending patent application is the combination of (1) a fully annealed aluminum foil having at least one bright, smooth electro-polished surface; (2) a first layer on said surface anodically formed from a chromic acid electrolyte, the resulting oxide being relatively porous; (3) a second layer on the first formed layer, anodically formed from a phosphate electrolyte, the resulting oxide being relatively dense; and (4) a conductive film of finely divided metal as the counterelectrode of the device. It is extremely important that the closure of a voltage-sensitive switch be reliable within a very narrow range.

It is an object of the invention to present a novel voltage-sensitive switch of high reliability;

It is another object of the invention to present a new process for preparing a voltage-sensitive switch; and

It is yet another object of the invention to present a process for determining the presence or absence of iron-containing impurity sites in aluminum.

### SUMMARY OF THE INVENTION

It has been determined that the closure of a voltage-sensitive switch results from oxide film breakdown at preferential sites. These sites can now be examined prior to breakdown by viewing the anodized aluminum under low power magnification. It has been discovered that if an aluminum electrode having iron-containing impurity sites is cleaned in a specific manner and then the cleaned surface treated with a hydroxyl-containing polar compound, preferably water, for a certain minimum period, then,

2

after anodization of the aluminum in a specific electrolyte, the iron-containing impurity sites are plainly visible.

The process for forming the voltage-sensitive switch can be summarized as follows: Chemically or electro-chemically polishing at least one surface of an aluminum electrode so as to leave the surface clean and smooth with only a surface oxide, the thickness of which is of the order of naturally occurring oxide, said surface having at least one iron-containing impurity site. Treating the cleaned surface with a hydroxyl-containing polar compound, preferably water, for a period sufficient to make the iron-containing impurity site latently visible. Anodizing the treated surface in an aqueous chromic acid solution to form an anodic oxide layer and make visible said iron-containing impurity site. The anodized surface is then rinsed to remove chromic acid and a counterelectrode is applied to the anodic oxide. In a preferred embodiment a second anodization in a phosphate electrolyte is performed to form a second dielectric which heals imperfections and partially fills the pores and voids of the first dielectric oxide.

The process can also be employed to determine the presence or absence of iron-containing impurity sites in aluminum by taking a sample of aluminum and performing the foregoing sequence of steps up through the step of rinsing to remove chromic acid. At this point visual inspection of the anodic oxide surface will reveal the presence or absence of iron-containing impurity sites. By this technique one can determine whether or not the aluminum represents raw material of minimally acceptable quality for the preparation of voltage-sensitive switches. If the process does not reveal at least one iron-containing impurity site per switch area, this aluminum should not be used in a voltage-sensitive switch. If the aluminum is iron-free, or substantially so, the aluminum will represent good raw material for aluminum capacitor manufacture.

The device of the present invention comprises an aluminum electrode having at least one comparatively clean surface; an aluminum oxide layer anodically formed on said surface, said oxide revealing at least one isolated iron-containing impurity site; and a counterelectrode applied to said dielectric oxide. In a preferred embodiment of the voltage-sensitive switch of the present invention, a second aluminum oxide heals imperfections and partially fills the pores of the first aluminum oxide. The device of the present invention can be prepared from fully annealed aluminum foil or from hard aluminum foil and a preferred counterelectrode for the present invention is silver.

### BRIEF DESCRIPTION OF THE DRAWING

The drawing represents a side view in section of part of a voltage-sensitive switch within the scope of the present invention.

The drawing shows a cross-sectional view of part of a voltage-sensitive switch 10. An aluminum electrode 12 has formed thereon an aluminum oxide dielectric 14. Said aluminum oxide has voids or pores 16 therein. A metal counterelectrode 18 is applied to the aluminum oxide dielectric. Located in the surface of the aluminum electrode is an iron-containing impurity site 20. The iron-containing impurity site is located in the center of a crater or depression 22. The region 24 bounded by the dotted lines represents the short or closure region of the device.

### DETAILED DESCRIPTION OF THE INVENTION

As previously indicated, it has been determined that the closure or shorting of a voltage-sensitive switch results from oxide film breakdown at preferential sites. By carefully cleaning and polishing the surface of an aluminum

electrode, followed by treating the cleaned and polished surface with a hydroxyl-containing polar compound, preferably water, and then by anodizing the aluminum in a specific electrolyte, the iron-containing impurity sites are made plainly visible. Electron probe micro-analysis of the breakdown sites has revealed a concentration of metallic impurities at these locations. The impurity sites were determined to contain iron with considerably lesser amounts of nickel and chromium. In order to prepare a reliable voltage-sensitive switch it is necessary that the aluminum electrode contains at least one iron-containing impurity site. The electrode must be cleaned with a reagent which removes all surface reaction product from the surface of the aluminum or at most which leaves a thin film somewhat akin to the comparatively thin natural oxide which forms on aluminum. This thin film can, for the purposes of the present invention, be ignored since it does not contribute materially to the resistance to physical breakdown of the unit. One such cleaning reagent is a perchloric acid-acetic anhydride solution. A chemical polishing solution which was not effective in properly cleaning an aluminum electrode is a phosphoric acid-nitric acid solution containing a small amount of cupric nitrate. Switches prepared from aluminum electrodes polished with this ineffective solution showed extremely high closures and no defect or impurity sites were observed after anodization of the aluminum electrodes.

After the aluminum electrode is properly cleaned the surface must be treated with a hydroxyl-containing polar compound, preferably water, for a sufficient length of time so that the iron-containing impurity sites in the aluminum will be rendered latently visible. The term "latently visible" means that on anodization of the aluminum electrode in the proper anodization electrolyte, the iron-containing impurity sites will be rendered plainly visible under low magnification. Water temperature and water flow will affect the time required to render the iron containing impurity sites latently visible. For example, using running distilled water at about 19° C., the impurity sites will become latently visible after about 1 minute. However, using static water, the time will be considerably longer. If the water temperature approaches 100° C., there is the likelihood of forming a hydrated film on the electrode which will result in the voltage-sensitive switch having extremely high and erratic closure voltages.

Investigation also has determined that only certain anodization electrolytes will properly develop or make plainly visible the iron-containing impurity sites. The anodization electrolyte should be of the type which produces a so-called porous electrolyte. Electrolytes of this type are represented by a chromic acid electrolyte or an oxalic acid electrolyte. An electrolyte such as ammonium dihydrogen phosphate does not reveal the presence of the iron-containing impurity sites and thus is not an effective anodization electrolyte for the initial anodic oxide layer of the voltage-sensitive switch of the present invention. While ammonium dihydrogen phosphate is not an effective electrolyte for the formation of the initial anodic oxide, it is a preferred electrolyte to be employed for the purpose of healing imperfections and partially filling the voids or pores which naturally occur in an oxide formed with an electrolyte such as chromic acid.

The counterelectrode of the voltage-sensitive switch can be any one of a number of prior art electrodes, however, a preferred counterelectrode is silver.

The starting material for the switch of the present invention as indicated must have at least one iron-containing impurity site per switch area. Commercially available 99.88 percent, 99.99 percent or 99.999 percent aluminum can be employed. While the aluminum either can be fully annealed or hard aluminum, it is preferred to use fully annealed material in order to avoid accidental cracking of the anodic oxide which is more common when hard foil is employed.

The following is a specific example of the preparation

of a voltage-sensitive switch within the scope of the present invention:

#### Example I

A length of 3 mil aluminum foil of 99.99% purity and known to contain iron-containing impurity sites is electro-polished in the solution made by mixing 138 milliliters of 60% perchloric acid (in water) with 483 milliliters of acetic anhydride. The foil is placed in the solution with one face of the foil opposite an aluminum cathode also immersed in this solution. An anodic current density of 10 milliamperes per square centimeter of said foil surface is passed through the system for 2½ minutes, the electrolyte being kept at about 23° C. and actively agitated. The foil is now much brighter in appearance. The polished sample is treated in running distilled water (flow rate 3 liters per minute) at 19° C. for a period of about 6½ minutes. The treated sample is anodized in a 1½% chromic acid electrolyte at 100° F. at 1 ma./cm.<sup>2</sup> for about 10 minutes. The anodized sample is then rinsed to remove the chromic acid. At this point, using a magnification of about 68 times, the iron-containing impurity sites are plainly visible as circular areas having a central dot which has been established as the site of the iron. The unit is then dried and a conductive film applied, using an electrically conductive silver paint such as that described in the Bureau of Standards circular 468, pages 5-7. Using a ramp circuit i.e. a circuit generating a linearly increasing voltage, the unit of the example was eventually subjected to a voltage which caused closure or shorting of the electrodes. Photomicrographic examination of the unit showed that the shorting of this device occurred at at least one of the iron-containing impurity sites.

#### Example II

In a preferred embodiment of the present invention the process of Example I is repeated but after anodization in chromic acid followed by rinsing, a second anodization step is carried out in a 0.01% ammonium dihydrogen phosphate electrolyte in order to heal imperfections and partially fill the pores which tend to naturally occur in the chromic acid-formed aluminum oxide. A preferred percentage range for the phosphate electrolyte is from 0.005 to 1.0%. The unit is then dried and a counterelectrode is added as in the foregoing example.

Units formed by the process of the present invention will reliably breakdown within an extremely narrow voltage range. No difficulty is experienced in preparing units which will reliably short at any predetermined voltage within the range of about 10 to 100 volts.

The chemical or electrochemical polishing agents contemplated herein must be capable of cleaning and smoothing the surface of the aluminum and leave no more than a surface oxide of not substantially greater thickness than that of the naturally occurring oxide. While the preferred polishing agent is a perchloric acid-acetic anhydride solution, other agents which will clean and polish aluminum to substantially the same degree can also be employed. In this respect reference is made to "The Electrolytic and Chemical Polishing of Metals" by W. J. McG. Tegart, published in 1959 by Pergamon Press.

In addition to water, which is preferred, other hydroxyl-containing polar compounds which may be employed herein are methyl alcohol, ethyl alcohol, alone or in combination or in combination with water.

The chromic acid anodization can be carried out in different concentrations of the acid. Chromic acid can be replaced by other electrolytes, such as oxalic acid, known to produce porous oxide films similar to that produced with chromic acid. The ammonium dihydrogen phosphate in the second anodization can be replaced by other electrolytes known to produce compact oxide films, such as diammonium hydrogen phosphate, sodium dihydrogen phosphate and disodium hydrogen phosphate.

The preferred counterelectrode metal is silver, however,

other metals and conductive films may substitute therefor.

Since it is obvious that many changes and modifications can be made in the above-described details without departing from the nature and spirit of the invention it is to be understood that the invention is not limited to said details except as set forth in the appended claims.

What is claimed is:

1. A method for determining the presence or absence of iron-containing impurity sites in aluminum comprising:

- (a) chemically or electrochemical polishing at least one surface of an aluminum sample so as to leave the surface clean and smooth with a surface oxide film of not substantially greater thickness than that of a naturally occurring aluminum oxide film produced under normal atmospheric conditions;
- (b) treating the cleaned surface with a hydroxyl-containing polar compound to render any iron-containing impurity site latently visible;
- (c) anodizing the treated surface in a porous oxide-forming electrolyte to form an aluminum oxide layer and make visible any iron-containing impurity sites; and
- (d) rinsing the anodized surface to remove electrolyte thereby exposing any iron-containing impurity sites.

2. The method of claim 1 wherein the electrochemical polishing is effected in a perchloric acid-acetic anhydride solution; the hydroxyl-containing polar compound is water; and the porous oxide-forming electrolyte is an aqueous chromic acid solution.

3. The method of claim 2 wherein said aluminum sample is aluminum foil; the electropolishing solution contains about 1 part 60% perchloric acid to from 2-4 parts acetic anhydride; the water-treating period is at least about one minute; and anodization is effected in a 0.01 to 10% chromic acid solution.

4. The method of claim 3 wherein said aluminum is fully annealed.

5. The method of claim 3 wherein said aluminum is hard foil.

6. A method for preparing a voltage-sensitive switch comprising the steps:

- (a) chemically or electrochemically polishing at least one surface of an aluminum electrode, so as to leave the surface clean and smooth with a surface oxide film of not substantially greater thickness than that of a naturally occurring aluminum oxide film produced under normal atmospheric conditions, said surface having at least one iron-containing impurity site;
- (b) treating the clean surface with a hydroxyl-containing polar compound to render said iron-containing impurity site latently visible;
- (c) anodizing the treated surface in a porous oxide-forming electrolyte to form an aluminum oxide layer

and make visible any iron-containing impurity sites;

- (d) cleaning the applied surface to remove electrolyte; and
- (e) applying an electrode to said anodic oxide.

5 7. The method of claim 6 wherein the electrochemical polishing is effected in a perchloric acid-acetic anhydride solution; the hydroxyl-containing polar compound is water; and the porous oxide-forming electrolyte is an aqueous chromic acid solution.

8. The method of claim 7 wherein said aluminum electrode is aluminum foil; the electropolishing solution contains about 1 part 60% perchloric acid to from about 2-4 parts acetic anhydride; the water-treating period is at least about one minute; and anodization is effected in a 0.01 to 10% chromic acid solution.

9. The method of claim 8 wherein after the chromic acid anodization, performing a second anodization in a phosphate electrolyte to form a second, compact dielectric which heals imperfections and partially fills the pores and voids in the chromic acid formed oxide.

20 10. The method of claim 9 wherein the second anodization is effected in a 0.005 to 1.0% aqueous electrolyte selected from the group consisting of ammonium dihydrogen phosphate, diammonium hydrogen phosphate, sodium dihydrogen phosphate and disodium hydrogen phosphate.

30 11. A voltage-sensitive switch comprising an aluminum electrode having at least one comparatively clean surface; a porous aluminum oxide layer anodically formed on said surface, at least one isolated iron-containing impurity site and said oxide layer plainly revealing said at least one isolated iron-containing impurity site; and a counterelectrode applied to said oxide.

12. The switch of claim 11 wherein said surface is an electropolished surface.

35 13. The switch of claim 12 wherein a second, compact aluminum oxide heals imperfections and partially fills the pores and voids of said porous aluminum oxide.

14. The switch of claim 13 wherein said electrode is fully annealed aluminum foil and said counterelectrode is silver.

40 15. The switch of claim 13 wherein said electrode is hard aluminum foil and said counterelectrode is silver.

#### References Cited

#### UNITED STATES PATENTS

|              |         |          |       |           |
|--------------|---------|----------|-------|-----------|
| 1,816,875    | 4/1931  | Siegmund | ----- | 317—230 X |
| 2,094,048    | 9/1937  | Siegel   | ----- | 317—230 X |
| 50 2,408,910 | 10/1946 | Burnham  | ----- | 317—230 X |

JAMES D. KALLAM, Primary Examiner

U.S. Cl. X.R.